

## 1

3,785,976

### PROCESS FOR PRODUCING ANIONIC METAL-CONTAINING SULFONATES

Mack W. Hunt, Ponca City, Okla., assignor to Continental Oil Company, Ponca City, Okla.

No Drawing. Filed May 7, 1971, Ser. No. 148,267  
Int. Cl. C10m 1/40

U.S. CL. 252—33

9 Claims

#### ABSTRACT OF THE DISCLOSURE

A process for producing anionic metal-containing sulfonates is disclosed wherein an anionic metal-containing acid is reacted with an oil-soluble sulfonic acid and an amino-alcohol in the presence of a nonvolatile carrier and water.

#### BACKGROUND OF THE INVENTION

This invention relates to anionic metal sulfonates. In one aspect the invention relates to a process for producing anionic metal sulfonates. In another aspect the present invention relates to a method for producing anionic metal sulfonates from anionic metal containing acids. In still another aspect the present invention relates to the production of anionic metal sulfonates by reacting an anionic metal containing acid with an oil-soluble sulfonic acid and an amino-alcohol in the presence of a nonvolatile carrier and water. In yet another aspect the present invention relates to the production of a boron-containing sulfonate from boric acid, an oil-soluble sulfonic acid, and an amino-alcohol containing from 1 to about 20 carbon atoms in the presence of a nonvolatile carrier and water.

#### BRIEF DESCRIPTION OF THE PRIOR ART

In recent years it has been found that superior standards for spectrographic equipment can be prepared from oil-soluble metal sulfonates and metal dispersions in such sulfonates by dissolving such material in predetermined quantities in a suitable solvent. Such standards have exhibited indefinite shelf life and any combination of metals can be combined without precipitation of the metal constituents.

Further, dispersions containing certain anionic metal sulfonates have acquired considerable importance as additives in fuels and lubricating oil. Such dispersions have been highly useful as additives to other materials where the problem of suspending insoluble waste materials formed in the utilization of the material and also the problem of corrosion inhibition is met. When the anionic metal sulfonates are employed as additives for use in internal combustion engine lubricating compositions such agents function to effectively disperse or peptize the insolubles formed by the fuel combustion, oil oxidation, or similar conditions obtained during the operation of the engine.

Thus, while the use of anionic metal sulfonates have been established and recognized, problems have been encountered in the production of such anionic metal sulfonates. For example, it has long been felt that because of boron's anionic properties sulfonates of such would have to be prepared as a binary mixture with another metal. As a result, the calcium carbonate dispersions were

## 2

converted to calcium borate dispersions and this product was used as the boron standard, such is not desirable because of the large quantities of other metals required to carry the boron. Therefore, a need has long been recognized for an improved process for the production of anionic metal sulfonates from readily available chemical compounds, and it is to such a process that the present invention is directed.

#### OBJECTS OF THE INVENTION

An object of the present invention is to provide an improved process for the production of anionic metal sulfonates. Another object of the present invention is to provide an economical, dependable, and efficient method for preparing anionic metal sulfonates from readily available chemical compounds. Another object of the present invention is to provide an improved method for the preparation of boron-containing sulfonate which is suitable as an analytical standard while at the same time providing an oil-soluble source of boron.

These and other objects, advantages, and features of the present invention would be apparent to those skilled in the art from a reading of the following detailed description.

#### SUMMARY OF THE INVENTION

According to the present invention I have found a process for producing anionic metal-containing sulfonates which basically involves reacting an anionic metal-containing acid with an oil-soluble sulfonic acid, and an amino-alcohol in the presence of a nonvolatile carrier and water.

Further, according to the invention, I have found that a boron-containing sulfonate can readily be prepared from boric acid by reacting the boric acid with an oil-soluble sulfonic acid and an amino-alcohol containing from 1 to about 20 carbon atoms, in a nonvolatile carrier and water. A volatile inert solvent can be incorporated with the oil-soluble sulfonic acid to reduce the viscosity of same and to facilitate the admixing of the oil-soluble sulfonic acid with the other constituents of the reaction mixture.

#### DESCRIPTION OF THE PREFERRED EMBODIMENTS

Anionic metal-containing sulfonates have been recognized as desirable analytical standards as well as oil-soluble additives for fuels and lubricants. However, problems have been encountered in producing such sulfonates. I have now found that anionic metal-containing acids can readily be converted to an anionic metal-containing sulfonate by a novel process which basically involves reacting the anionic metal-containing acid with an oil-soluble sulfonic acid and an amino-alcohol containing 1 to about 20 carbon atoms, in the presence of a nonvolatile carrier, and water. The present invention can be carried out in either a batch-type process or a continuous process. However, for the sake of simplicity, the process of the present invention will be described as a batch-type process.

In a batch-type process the anionic metal-containing acid, the amino-alcohol, the oil-soluble sulfonic acid, the

nonvolatile carrier, and the water are charged to a reaction vessel which is equipped with stirring and heating means. The amount of reactants employed will vary widely but the amino-alcohol constituent is added in at least a stoichiometric amount based on the oil-soluble sulfonic acid whereas the anionic metal-containing acid is added in about a stoichiometric amount based on the amount of amino-alcohol employed. The amount of nonvolatile carrier employed is dependent solely upon the viscosity of the product desired. Generally, however, the amount of nonvolatile carrier will range from about 10 to 70 weight percent, based on the total reaction mixture. Likewise, the amount of water employed can vary broadly but will generally be present in an amount ranging from about 5% to 50% by weight. Once the reactants have been introduced into the reaction vessel the reactants are thoroughly agitated and the reaction mixture is heated to the reflux temperature which will generally be within the range of about 50 degrees C. to about 125 degrees C. The heating period is carried out slowly so as to be over a period of time from about 1 hour to 10 hours. During this heating period the volatile components, including the water are removed. An additional amount of the nonvolatile carrier compound can then be added to the reaction mixture and the mixture heated to a temperature within the range of about 125 degrees C. to 175 degrees C. The amount of additional nonvolatile carrier employed will vary widely but will generally range from about 10 to 50 percent by weight of the amount of the volatile solvent originally employed. During this second heating step the product is stripped with an inert gas, such as nitrogen, carbon dioxide, or helium for a period of time ranging from about 20 minutes to 3 hours.

Additional purification steps, such as polish filtering the product can be employed. In addition when a highly pure product is desired one should use distilled water as the water constituent. The product obtained contains from about 10 to 90 weight percent of the anionic metal-containing sulfonate in the nonvolatile carrier. In addition it should be evident that other inert solvents can be employed to facilitate the mixing of the reactants during both the initial heating period and the second or subsequent heating period. For example, the oil-soluble sulfonic acid can be diluted with from about 10 to 80 weight percent of a volatile solvent such as petroleum naphtha hydrocarbons, such as hexane, heptane, octane, toluene, benzene or xylene. The use of such volatile solvents is merely to enhance the mixability of the sulfonic acid constituent into the reaction mixture and the solvent will be stripped due to the steps incurred in the process as described above.

In practicing the process of the present invention for the preparation of anionic metal sulfonates from anionic metal-containing acids, any suitable anionic metal-containing acid can be employed. Examples of suitable anionic metal constituents which can be employed in the acid are boron, silicon, phosphorus, arsenic, selenium and vanadium. Desirable results have been obtained wherein boric acid is employed as the anionic metal-containing acid.

The amino-alcohols which are suitable for use in the process of the present invention are represented by the general formula  $NR_3$  wherein R is H,  $-C_nH_{2n}OH$ , OH,  $C_nH_{2n+1}$ ,  $NH_2$ , and mixtures thereof and n is an integer of from 1 to 20. Desirable results have been obtained wherein the alkyl radical contains from 1 to about 8 carbon atoms. Further, the amino-alcohol is one in which the anionic metal-containing acid constituent and the oil-soluble sulfonic acid have an appreciable solubility. Examples of suitable amino-alcohols falling within the above-defined limits are: ethanol amine, diethanol amine, triethanol amine, propanol amine, dipropanol amine, 2-methyl 2-amino propanediol, 2,3-dimethyl 2-amino 1,4-butanediol, butyl-amino alcohols, hepta-, hexa-amino

alcohols, etc., branched amino diols, branched amino triols, etc.

Suitable oil-soluble hydrocarbon sulfonic acids include alkane sulfonic acid, aromatic sulfonic acid, alkaryl sulfonic acid, dialkaryl sulfonic acids, aralkyl sulfonic acid, and the natural petroleum mahogany sulfonic acids. The mahogany sulfonic acids include any of those materials which may be obtained by concentrated or fuming sulfuric acid treatment of petroleum fractions, particularly the higher boiling lubricating oil distillates and white oil distillates. The higher molecular weight petroleum oil-soluble mahogany sulfonic acids are condensed-ring compounds, which condensed-rings may be aromatic or hydroaromatic in nature. Alkyl and/or cycloalkyl substituents may be present in the mahogany sulfonic acids.

The term "oil-soluble sulfonic acids," as used herein, refers to those materials wherein the hydrocarbon portion of the molecule has a molecular weight in the range of about 300 to about 1,000. Preferably, this molecular weight is in the range of about 370 to about 700. These oil-soluble sulfonic acids can be either synthetic sulfonic acids or the so-called mahogany or natural sulfonic acids. The term "mahogany sulfonic acids" refers to those materials which are prepared by sulfonation of hydrocarbon feedstocks which are prepared synthetically. The synthetic sulfonic acids can be derived from either alkyl or alkaryl hydrocarbons. In addition, they can be derived from hydrocarbons having cycloalkyl (i.e., naphthenic) groups in the side chains attached to the benzene ring. The alkyl groups in the alkaryl hydrocarbons can be straight or branched chain. The alkaryl radical can be derived from benzene, toluene, ethyl benzene, xylene isomers, or naphthalene.

An example of a hydrocarbon feedstock which has been particularly useful in preparing synthetic sulfonic acids is a material known as postdodecylbenzene. Postdodecylbenzene is a bottoms product of the manufacture of dodecylbenzene. The alkyl groups of postdodecylbenzene are branched chain. Postdodecylbenzene consists of monoalkylbenzenes and dialkylbenzenes in the approximate mole ratio of 2:3 and has typical properties as follows:

|                                   |        |
|-----------------------------------|--------|
| Specific gravity at 38 degrees C. | 0.8649 |
| Average molecular weight          | 385    |
| Percent sulfonatable              | 88     |
| ASTM D-158 Engler:                |        |
| I.B.P. degrees F.                 | 647    |
| 5 degrees F.                      | 682    |
| 50 degrees F.                     | 715    |
| 90 degrees F.                     | 760    |
| 95 degrees F.                     | 775    |
| F.B.P. degrees F.                 | 779    |
| Refractive index at 23 degrees C. | 1,4900 |
| Viscosity at:                     |        |
| -10 degrees C., centistokes       | 2800   |
| 20 degrees C., centistokes        | 280    |
| 40 degrees C., centistokes        | 78     |
| 80 degrees C., centistokes        | 18     |
| Aniline point, degrees C.         | 69     |
| Pour point, degrees F.            | -25    |

An example of another hydrocarbon feedstock which is particularly useful in preparing synthetic sulfonic acids is a material referred to as "dimer alkylate." "Dimer alkylate" has a long, branched-chain alkyl group. Briefly described, dimer alkylate is prepared by the following steps:

- (1) dimerization of a suitable feedstock, such as cat poly gasoline.
- (2) alkylation of an aromatic hydrocarbon with the dimer formed in step (1).

Preferably, the dimerization step uses a Friedel-Crafts alkylation sludge as the catalyst. This process and the resulting product are described in U.S. Pat. No. 3,410,925.

An example of another hydrocarbon feedstock which is particularly useful for preparing synthetic sulfonic acids which can be used in my invention is a material which I refer to as "NAB Bottoms." NAB Bottoms are predominantly di-n-alkyl aromatic hydrocarbon wherein the alkyl groups contain from 8 to 18 carbon atoms. They are distinguished primarily from the preceding sulfonation feedstocks in that they are straight chain and contain a large amount of di-substituted material. A process of preparing these materials and the resulting product are described in application Ser. No. 62,211, filed Aug. 7, 1970, and being a continuation-in-part of application Ser. No. 529,284, filed Feb. 23, 1966, and now abandoned. Application Ser. Nos. 62,211 and 529,284 have the same assignee as the present application. The product is also described in U.S. Pat. No. 3,288,716, which is concerned with an additional use for the product, other than sulfonation feedstock. Another process of preparing these materials is described in application Ser. No. 53,352, filed Aug. 6, 1970, and having the same assignee as the present application. Application Ser. No. 53,352 is a continuation-in-part of application Ser. No. 529,284. Still another process of preparing a di-n-alkaryl product is described in application Ser. No. 104,476, filed Jan. 7, 1971, which is a continuation-in-part of application Ser. No. 521,794, filed Jan. 20, 1966, and now abandoned.

In order to make my disclosure even more complete, U.S. Pat. No. 3,410,925 and application Ser. Nos. 53,352; 62,211 and 104,476 are made a part of this disclosure.

In addition to the sulfonic acids derived from the foregoing described hydrocarbon feedstock, examples of other suitable sulfonic acids include the following: mono- and poly-wax-substituted naphthalene sulfonic acid, dinonyl naphthalene sulfonic acid, diphenyl ether sulfonic acid, naphthalene disulfide sulfonic acid, dicetyl thianthrene sulfonic acid, dilauryl betanaphthol sulfonic acid, dicapryl nitronaphthalene sulfonic acid, unsaturated paraffin wax sulfonic acid, hydroxy substituted paraffin wax sulfonic acid, tetraamylene sulfonic acid, mono- and poly-chloro-substituted paraffin wax sulfonic acid, nitrosoparaffin wax sulfonic acid, cycloaliphatic sulfonic acid such as lauryl-cyclohexyl sulfonic acid, mono- and poly-wax-substituted cyclohexyl sulfonic acid, and the like.

In order to disclose more clearly the nature of the present invention, the following example is given. It is to be understood that the example is for illustrative purposes only and is not to be construed as undue limitations upon the invention.

#### Example I

A twelve-liter, 3-neck flask was charged with the following:

|                                      | G.    |
|--------------------------------------|-------|
| Sulfonic acid <sup>1</sup> in hexane | 5,000 |
| Triethanol amine                     | 810   |
| Distilled water                      | 1,000 |
| Boric acid                           | 355   |
| 80 pale oil                          | 1,000 |

<sup>1</sup> A disproportionated dialkyl benzene sulfonic acid having the following properties:

|                                   |                   |
|-----------------------------------|-------------------|
| Total acidity                     | 1.015 meqs./gm.   |
| Sulfonic acidity                  | 0.953 meqs./gm.   |
| Percent non vol.                  | 52.4%             |
| Molecular weight of sulfonic acid | 500 grams (avg.). |
| Percent hexane                    | 47.6%.            |

The above was mixed well and heated to reflux. Reflux conditions were maintained for about one hour and then solvent was removed to 100 degrees C. Then, another 1,500 g. of 80 pale oil was added. Heating was continued to 150 degrees C. and the product was stripped with nitrogen for about 45 minutes. The product was polish filtered. The product contained 1.0 percent boron.

#### Example II

A one-liter, 3-neck flask was charged with:

|                                      | G.   |
|--------------------------------------|------|
| Sulfonic acid <sup>1</sup> in hexane | 100  |
| 2-methyl, 2-amino propanol           | 10.7 |
| 80 pale oil                          | 56   |
| Distilled water                      | 50   |
| Boric acid                           | 7.1  |

<sup>1</sup> A disproportionated dialkyl benzene sulfonic acid having the following properties:

|                     |                 |
|---------------------|-----------------|
| Total acidity       | 1.089 meqs./gm. |
| Sulfonic acidity    | 1.035 meqs./gm. |
| Percent nonvolatile | 47.1%.          |
| Percent hexane      | 52.9%.          |

Molecular weight of sulfonic acid 489 grams (avg.).

The above was well mixed and the mixture was heated slowly and the solvents were removed to 150 degrees C. (over about 2 hours). The product became bright and clear at about 100 degrees C. At 150 degrees C. the mixture was stripped with carbon dioxide for about 20 minutes. The product was polish filtered and determined to contain 1.0 percent boron.

The above example clearly indicates the preparation of an anionic metal sulfonate by the process of the present invention.

Having thus described the invention, I claim:

1. A process for producing anionic metal sulfonates which comprises:

(a) admixing an anionic metal-containing acid, wherein the metal constituent of said acid is selected from the group consisting of boron, arsenic, selenium and vanadium, an amino-alcohol having from 1 to about 20 carbon atoms, an oil-soluble sulfonic acid, from about 5 to 50 weight percent water and from about 10 to 70 weight percent nonvolatile carrier to form a reaction mixture, said anionic metal-containing acid being present in about a stoichiometric amount with said amino-alcohol and said amino-alcohol being present in at least a stoichiometric amount with said oil-soluble sulfonic acid;

(b) heating said reaction mixture to the reflux temperature of said mixture and then removing the volatile components therefrom thereby forming a stripped mixture;

(c) heating said stripped mixture to a temperature in the range of about 125 to about 175 degrees C. for a period of time ranging from about 20 minutes to 2 hours; and

(d) recovering the nonvolatile carrier containing from about 10 to 90 weight percent anionic metal sulfonate.

2. The process of claim 1 which includes the step of admixing from about 10 to 50 weight percent of additional nonvolatile carrier to said stripped mixture, said carrier being the same employed in said reaction mixture.

3. The process of claim 2 wherein said amino-alcohol is represented by the general formula  $NR_3$  wherein R is selected from the group consisting of H,  $-C_nH_{2n}OH$ ,  $OH$ ,  $C_nH_{2n+1}$ ,  $NH_2$  and mixtures thereof and wherein n is an integer of from 1 to 20.

4. The process of claim 3 wherein said alkyl radical of said amino-alcohol contains from 1 to about 8 carbon atoms and wherein said reflux temperature is from about 50 to 125 degrees C. and is carried out slowly over a period of time of from about 1 hour to 10 hours.

5. The process of claim 4 which includes the step of contacting said stripped mixture during the heating of same with an inert gas for a period of time of from about 20 minutes to 3 hours.

6. The process of claim 5 which includes the step of polish filtering the nonvolatile carrier-anionic metal sulfonate product.

7. The process of claim 6 wherein said water is distilled water, and said nonvolatile carrier is a pale oil.

8. The process of claim 7 wherein said amino-alcohol is triethanol amine and said oil-soluble sulfonic acid is an dialkaryl sulfonic acid diluted with from about 10 to 80 weight percent hexane, said alkaryl sulfonic acid having a molecular weight in the range of about 300 to 1000.

9. The process of claim 7 wherein said amino-alcohol is 2-methyl, 2-amino propanediol and said oil-soluble sulfonic acid is an alkaryl sulfonic acid diluted with from about 10 to 80 weight percent hexane, said alkaryl sulfonic acid having a molecular weight in the range of about 370 to 700.

## References Cited

## UNITED STATES PATENTS

|           |         |                  |       |          |
|-----------|---------|------------------|-------|----------|
| 3,219,580 | 11/1965 | Stratton         | ----- | 252—33   |
| 2,889,279 | 6/1959  | Carlyle et al.   | ----- | 252—33   |
| 3,535,242 | 10/1970 | Hashimoto et al. | ----- | 252—33   |
| 2,606,872 | 8/1952  | Gasser et al.    | ----- | 252—33.4 |
| 2,947,694 | 8/1960  | Gragson          | ----- | 252—33.4 |
| 3,277,002 | 10/1966 | Hunt et al.      | ----- | 252—33.4 |

DANIEL E. WYMAN, Primary Examiner

I. VAUGHN, Assistant Examiner

U.S. CL. X.R.

15 44—68, 76; 252—46.3; 260—429 K, 440, 462, 607